

# UNITED STATES PATENT OFFICE.

EUGEN RECK, OF CHARLOTTENBURG, GERMANY, ASSIGNOR TO FREESES PATENT  
EISENSCHUTZ UND SCHRAUBENWELLENBEKLEIDUNG FUR SCHIFFE G. M. B. H.,  
OF CHARLOTTENBURG, GERMANY.

COATING FOR THE PRESERVATION OF WOOD, PASTEBOARD, MASONRY, LEATHER,  
SHEET IRON, ETC.

1,418,172.

Specification of Letters Patent. Patented May 30, 1922.

No Drawing.

Application filed January 6, 1921. Serial No. 435,564.

To all whom it may concern:

Be it known that I, EUGEN RECK, a citizen of the German Republic, and resident of Charlottenburg, Germany, have invented 5 certain new and useful Improvements in an Improved Coating for the Preservation of Wood, Pasteboard, Masonry, Leather, Sheet Iron, Fabric, and the like (for which I have made application in Germany Oct. 25, 1919), 10 of which the following is a specification.

The object of this invention is to provide an improved coating for the preservation of wood, pasteboard, masonry, leather, sheet iron, fabric and the like.

15 The improved coating is composed of minium and tar, with the addition of a suitable diluting product and colouring substances if desired. A mixture of 3 to 5 parts of minium and 1 to 2 parts of wood tar 20 with the addition of turpentine or its equivalent has been found particularly convenient. For the ingredients mentioned, their chemical equivalents may be substituted, for instance zinc-white may be substituted, for minium and xylidin for turpentine.

25 The coating has properties which could not be expected from the same. The coating without diluting liquid composed of 4 to 5 parts of minium and 1 part of wood tar has been proposed heretofore merely for the purpose of coating screw-shafts of ships against rust.

30 The surface coated with the improved mass and treated with a brush becomes bright in a very particular way, for instance the surface of sheet iron. If the surface is coated twice, it will become bright and brilliant like enamel.

35 It is a very important feature that the coating combines with the body to be protected and forms an insoluble compound, whereby a compact non porous surface and therefore a high grade protection of the 40 coated body against moistness, bacilli and like rotting agents will be obtained. Thus the coating mass forms a superior preservative means. The tenacious coherence of the 45 particles forming the surface of the coating is such that for instance a piece of sheet iron coated with the improved mass may be 50 bent through an angle of 180°, that is nearly

folded upon itself, and then straightened again, without the slightest crack to be produced on the surface thereof. 55

It may be said that the insoluble compound is produced—at least with porous bodies such as wood, pasteboard, leather and the like—by the fact that the mass enters the pores thereof whereby an extremely efficient surface adhesion will be secured. The coating mass and the mass of the body are rather melted together with the result that a new body will be formed. Thus pasteboard coated with the improved mass has 60 in cross section three distinct layers, viz, the layer of pasteboard, a layer of pasteboard impregnated with the coating mass, and the surface layer. Such pasteboard is 65 designed according to this invention to be 70 sold as a new article of manufacture, for instance as a substitute for press-spahn commonly used in electrical industry. Owing to its particular treatment press-spahn is 75 expensive. Pasteboard coated on one or both sides with the improved mass is cheaper and has high grade insulating properties, which has been found by practical experiments. And as the coating mass, as 80 already stated, forms a superior protecting means against moistness, it may also be used in electrical industry in cases where the use of press-spahn is undesirable or impossible owing to the fact that it is capable of absorbing moistness. Furthermore owing 85 to the process used in its manufacture press-spahn is very rigid, whilst pasteboard treated with the improved coating remains 90 yieldable.

Owing to these important properties the 90 improved coating mass may be applied or used on a large scale. Besides the scope of application described above, said mass may also be used in the manufacture of bright pasteboard for book bindings, particular 95 boardings and pasteboard trunks. Fabric treated with the improved coating mass becomes watertight, and therefore it may be advantageously used for impregnating tents, tilts and the like. 100

The combination of the coating mass with sheet iron which resists to all practical conditions make the said mass convenient for coating toys of sheet metal.

Leather treated with the improved coating mass has the nature and appearance of varnished leather.

It will be obvious that it is impossible to 5 enumerate all the possibilities of uses of the improved coating mass and therefore we wish it to be understood that applications which are not mentioned in this specification are also contemplated by my invention.

10 Having now fully described my said invention, what I claim and desire to secure by Letters Patent, is:

1. An improved coating for the preservation of wood, pasteboard, masonry, leather, 15 sheet iron, fabric and the like, composed of minium, tar and a diluting liquid mixed together, substantially as set forth.

2. An improved coating for the preservation of wood, pasteboard, masonry, leather, 20 sheet iron, fabric and the like, composed of minium, tar, diluting liquid and coloring substances mixed together, substantially as set forth.

3. An improved coating for the preservation 25 of wood, pasteboard, masonry, leather, sheet iron, fabric and the like, composed of 2-5 parts of minium and 1-2 parts of wood-tar, mixed with a diluting liquid, substantially as set forth.

30 4. As a new article of manufacture pasteboard coated with a mixture of minium, wood-tar and diluting liquid, substantially as set forth.

5. As a new article of manufacture, paste-

board coated on both sides with a mixture 35 of minium, wood-tar and diluting liquid, substantially as set forth.

6. As a new article of manufacture, pasteboard coated with a mixture of 2-5 parts of minium, 1-2 parts of wood-tar and a 40 diluting liquid, substantially as set forth.

7. An improved coating for the preservation of wood, pasteboard, masonry, leather, sheet iron, fabric, and the like, composed of minium with one-half the quantity 45 thereof of wood-tar mixed together with a diluting liquid.

8. An improved coating for the preservation of wood, pasteboard, masonry, leather, sheet iron, fabric, and the like, composed of minium, wood-tar and diluting 50 liquid mixed together.

9. An improved coating for the preservation of wood, pasteboard, masonry, leather, sheet iron, fabric, and the like, composed of three fifths parts of minium, and approximately one part of wood-tar mixed 55 with a diluting fluid.

10. As an article of manufacture, pasteboard coated with a mixture of three fifths 60 parts of minium, approximately one part of wood-tar, and a diluting liquid.

In testimony whereof I have hereunto set my hand in presence of two witnesses.

EUGEN RECK.

Witnesses:

C. GEORGES DELBROUCK,  
HENRI DETMET.